

# UNITED STATES PATENT OFFICE.

SAMUEL CHARLES LANSDOWN, OF MELBOURNE, AND PHILIP MAGNUS, OF NORTH FITZROY, NEAR MELBOURNE, VICTORIA, AUSTRALIA.

## METHOD FOR THE TREATMENT AND UTILIZATION OF SCRAP OR WASTE LEATHER.

1,405,600.

Specification of Letters Patent. Patented Feb. 7, 1922.

No Drawing.

Application filed October 14, 1918. Serial No. 258,108.

(GRANTED UNDER THE PROVISIONS OF THE ACT OF MARCH 3, 1921, 41 STAT. L., 1313.)

To all whom it may concern:

Be it known that we, SAMUEL CHARLES LANSDOWN, of Empire Building, Flinders Street, Melbourne, Victoria, Australia, and PHILIP MAGNUS, of 333 Rae Street, North Fitzroy, near Melbourne, Victoria, Australia, have invented a new and useful Improvement in Methods for the Treatment and Utilization of Scrap or Waste Leather, (for which we have filed application in Australia, application No. 5544, Oct. 19, 1917,) of which the following is a specification.

At the present time scrap leather left over from the manufacture of different leather articles is wasted and it is with the object of regenerating this waste product so as to use the same as a commercial and marketable product that our invention has been devised.

After treatment as hereinafter described, the resultant product can be cut into various lengths, sizes and shapes, so as to be utilized for the purpose for which leather is at present used, but principally for boot and shoe leather. In achieving the object of our invention we first of all take any predetermined quantity of scrap or waste leather and by the aid of suitable machinery grind or reduce the same to a coarse powder. The powdered scrap leather is then placed in a shallow tank of tepid water containing a percentage say about two of oxalic acid.

The object of using oxalic acid is for the purpose of cleansing the powdered waste leather and destroying any impurities that may be contained therein. The mass is then gently stirred and placed in a further tank for further washing.

The admixture of oxalic acid and water, besides cleansing the scrap powdered leather forms it into a gelatinous mass.

It is then taken from the second tank and allowed to slowly dry in a shady place.

The next step in the process is to mix with the cleansed powdered scrap leather, an adhesive which will have the purpose of combining the various particles together and after pressure to form a solidified mass of great strength and to render waterproof. It is also necessary to add to the powdered mass certain chemicals, which will have the effect of keeping the manufactured leather

in an exceedingly dry state and in a state impervious to water or mould.

To manufacture an adhesive or cement for binding the particles together and rendering the manufactured article waterproof we mix with the gelatinous mass of scrap leather the following chemicals, in or about the proportions enumerated.

(1) Liquid glue 85%; (2) boiled linseed oil 10%; (3) carbolized oil 2½%; (4) oil of cloves 2½%.

The two former chemicals act as an adhesive and water-proofing, whilst the latter two will keep the regenerated leather when manufactured in a dry state.

The chemicals are intermixed together whilst in a hot state which is occasioned by the reduction of the solid glue to a liquid state and a sufficient quantity of the cleansed ground leather is mixed therewith to form a plastic mass. When in this state the mass is run or placed into suitable moulds of any desired shape or size and submitted to hydraulic pressure of about 4 tons per square inch. The pressure as will be understood, forms the plastic mass into solid sheets or pieces.

The sheets are then removed from the moulds and allowed to dry in the atmosphere, the sheets soles or heels and the like can be manufactured into any size or shape for any specific purpose.

### Claim:

An improved method of and means for the treatment and utilization of scrap or waste leather consisting of reducing the same to a coarse powder, cleansing the powdered leather with oxalic acid adding thereto an adhesive and drying composition consisting of liquid glue, boiled linseed oil, carbolized oil and oil of cloves in or about the proportions set out substantially as herein described.

In witness whereof we have signed this specification in the presence of two witnesses this 10th day of August, 1918.

SAMUEL CHARLES LANSDOWN.

PHILIP MAGNUS.

### Witnesses:

WILLIAM FRANCIS CLAPPEL,  
VICTOR MAGNUS.